

## 1

3,305,410

## HEAT TREATMENT OF ALUMINUM

George Robert Sublett, Sheffield, and Michael Waldemar Fien, Florence, Ala., assignors to Reynolds Metals Company, a corporation of Delaware  
No Drawing. Filed Apr. 24, 1964, Ser. No. 362,493  
12 Claims. (Cl. 148—159)

This invention relates to a novel method for improving the corrosion resistance of aluminum base alloys. More particularly, the invention concerns a novel two-stage method of aging such aluminum base alloys subsequent to their solution heat treatment.

Heat-treatable aluminum base alloys, especially the aluminum-copper and the aluminum-zinc-magnesium copper alloys, are extensively employed by the aircraft and aerospace industries. In these and other applications, such alloys must meet stringent corrosion requirements. However, experience has shown that these alloys frequently exhibit a tendency toward the development of undesirable forms of corrosion, such as intergranular corrosion which results in drastic reduction of the mechanical properties of these alloys, and stress corrosion which may result in sudden and possibly catastrophic failures.

Previous attempts to alleviate this tendency to corrode have either failed to adequately improve corrosion resistance or have done so only at the expense of reducing mechanical properties. An object of the invention was, therefore, to find a way of minimizing the tendency toward intergranular and stress corrosion in the case of artificially aged aluminum base alloys; and a further object was to find an optimum aging procedure, which would change the tendency toward intergranular corrosion to a shallow, pitting type of attack when the alloy was exposed to accelerated corrosion, and which would also produce typical mechanical properties.

The conventional practices previously known may be classified in three categories: (1) "constant temperature aging treatments," in which the metal is aged at a suitable temperature which is not intentionally varied during the aging operation; (2) "interrupted aging treatments," in which the metal is aged at one temperature for a period of time, then cooled to room temperature, and thereafter is heated at a higher temperature for an additional period of time; and (3) "progressive aging treatments," in which the metal is aged at one temperature for a period of time, then is heated and held at a higher temperature for an additional period of time.

In accordance with the invention, it has been found that the tendency toward intergranular and stress corrosion of aluminum base alloys of the type which are susceptible to artificial aging can be minimized by performing the aging treatment in two stages, whereby the first stage is conducted at a higher temperature than the second stage. After the first stage the metal may be either cooled directly to the second stage temperature, or cooled to room temperature and subsequently reheated to the temperature of the second stage of the treatment, the former practice ordinarily being preferred because it reduces the overall processing time. Thus, for example, in the case of 2024 alloy, which is a copper-bearing aluminum base alloy and will serve for purposes of illustration, a typical high-low aging treatment in accordance with the invention is to maintain the alloy at about 400° F. for about three hours, followed by holding the alloy at about 300° F. for about ten hours. For comparison purposes, the conventional aging treatment normally specified for 2024 alloy (Military Specification MIL-H-6088C, October 15, 1962) consists of a constant aging temperature of 370° to 380° F. for a time of 7 to 16 hours, the aging time varying with the temper desired. Thus, the first stage aging temperature in accordance with the present inven-

## 2

tion is preferably higher than the usual constant-temperature aging practice for the alloy, and the second stage temperature is ordinarily lower than the conventional aging temperature.

By carrying out the aging practice in this high-low sequence, resistance to intergranular and stress corrosion is appreciable improved. The initial high temperature is believed to have the effect to starting a controlled precipitation of the strengthening constituents in a generally uniform manner throughout the alloy, with the result that concentration of precipitated constituents at the grain boundaries (and consequent depletion thereof in the adjoining portions) is avoided or at least minimized. The final aging at a reduced temperature completes the precipitation begun at the favorable locations, without causing the reduction in mechanical properties which ordinarily is associated with long aging times at higher temperatures.

The method of the invention is applicable to a variety of heat-treatable aluminum base alloys, including copper-bearing alloys as well as zinc-bearing alloys. The conventional solution heat treating practice for such alloys involves heating at a temperature which ranges from about 840° F. to 1050° F., followed by water quenching.

The novel process of the invention produces particularly favorable results with aluminum base alloys which are low in silicon content, preferably below about 0.5% by weight. Thus, in the copper-bearing alloy series, alloy 2024, which has a silicon content of 0.50% maximum is virtually completely protected against intergranular corrosion by the method of the invention, whereas alloy 2017, which has 0.8% maximum silicon content and ordinarily contains more silicon than 2024 alloy, responds less favorably.

In the case of alloy 2024, the most favorable high-low aging treatment comprises maintaining the alloy in a first aging step at a temperature of from about 375° F. to about 425° F. for about 3 hours, and in a second aging step, maintaining the alloy at a temperature from about 275° F. to about 325° F. for about 10 hours. The preferred treatment for alloy 2024 is a first step aging at 400° F. for 3 hours, followed by a second step aging at 300° F. for 10 hours. The time periods for the two steps can vary somewhat according to the temperature used. Thus, the aging time can be shorter for a temperature of 425° F. than the 3 hour period for 400° F.

In the case of alloy 2017, it has been found that a first aging step at 450° F. for about 2 hours, followed by a second aging step at 325° F. for about 4 hours, yielded satisfactory results. These temperatures are similarly subject to variations in range of about 25° F. upward or downward.

In the case of alloy 7075, the preferred treatment is a first aging step at about 350° F. for about 5 hours, followed by a lower temperature aging step at about 250° F. for about 10 hours. The temperature ranges for zinc-bearing alloys in general are about 325–400° F. for the initial aging step, and about 200–300° F. for the second step.

In evaluating the improvement in intergranular corrosion produced by the method of the invention, there may be employed the procedure outlined in Military Specification MIL-H-6088C, October 15, 1962. In this procedure, each sample is immersed for 1 minute in an etching solution at 200° F. to produce a uniform surface condition. The etching solution is composed of 50 ml. 70% HNO<sub>3</sub>, 5 ml. 48% HF, balance distilled water. After this etching treatment, the sample is rinsed in distilled water, immersed for 1 minute in concentrated HNO<sub>3</sub> (70%) at room temperature to remove surface plated copper, rinsed in distilled water and allowed to dry. The sample is then corroded by immersion in a minimum of 30 ml. per square inch of surface area of a solution hav-

ing the composition: Sodium chloride 57 grams, hydrogen peroxide (30%) 10 ml., diluted to 1 liter with distilled water. The immersion period is six hours. At the end of the immersion period, the sample is removed, washed and dried. A cross-section specimen is cut and subjected to microscopic examination at 100 to 500 diameters magnification. The microscopic examination is made both before and after etching the specimen, using a metallurgical microscope. The etching is done by immersion for 6 to 20 seconds in a solution having the composition: 70%  $\text{HNO}_3$ , 2.5 ml., HCl (conc.) 1.5 ml., 48% HF 1 ml., distilled water 95 ml. There should be no evidence of excessive intergranular corrosion.

The heat-treated test samples are also tested for tensile strength, yield strength, and elongation properties.

The following examples illustrate the practice of the novel method of the invention, but are not to be considered as limiting:

#### EXAMPLE 1

##### *High-low aging of alloy 2024*

A length of (solution heat treated) 2024 alloy rod, 1½ inches in diameter, was cut into tensile strength and corrosion test specimens. The corrosion specimens consisted of ¾ inch disc, cut in half and machined along the cut face. The tensile strength specimens were standard size. The chemical analysis of the rod was Si 0.15, Fe 0.30, Cu 4.20, Mn 0.60, Mg 1.48, balance substantially Al.

Various individual specimens were subjected to aging cycles as shown in Table 1. The aged tensile strength specimens were tested for tensile strength, yield strength, and elongation, using standard tests. The corrosion specimens were subjected to the standard accelerated  $\text{NaCl}-\text{H}_2\text{O}_2$  corrosion test, mounted, etched and examined microscopically, as described above. The results are summarized in Table 1.

TABLE 1

| Sample No. | 1st Step Aging Cycle | 2nd Step Aging Cycle | Tensile (k.s.i.) | Yield (k.s.i.) | Elongation in 2 inch |
|------------|----------------------|----------------------|------------------|----------------|----------------------|
| 1-----     | 400° F., 3 hrs-----  | 300° F., 17 hrs----- | 71.7             | 65.5           | 10                   |
| 2-----     | do-----              | 300° F., 10 hrs----- | 72.7             | 65.2           | 10                   |
| 3-----     | 375° F., 10 hrs----- | do-----              | 71.2             | 64.7           | 9                    |

Of the specimens shown in the table, No. 2 had received the optimum aging treatment. Metallographic examination showed the precipitate was finely divided throughout the matrix. The mechanical properties of all three samples were very good, and exceeded the minimum specification properties (66.0 k.s.i. tensile strength, 58 k.s.i. yield strength, and 5% elongation).

Corrosion specimens corresponding to those in Table 1 were tested, and the corrosion depth measured. The results are set forth in Table 2:

TABLE 2

| Sample No. | Depth (mils), Avg. | Depth (mils), Max. | Type of Corrosion |
|------------|--------------------|--------------------|-------------------|
| 1-----     | 3.4                | 6.1                | Pitting.          |
| 2-----     | 3.4                | 5.3                | Do.               |
| 3-----     | 3.5                | 7.5                | Do.               |

#### EXAMPLE 2

The purpose of this example was to provide two sets of comparative corrosion tests in aging alloy 2024, the

first employing the standard aging treatment of 13 hours at 375° F., the control group, and a second series according to the preferred method of the invention, aging at 400° F. for 3 hours followed by a second aging at 300° F. for 10 hours.

Different diameter 2024 rods, ranging from 2.5" to 3.5" diameter were cut into corrosion specimens. The corrosion tests were carried out as specified previously. Average and maximum depths of corrosion and type of corrosion were determined.

The results as shown in Table 3 clearly demonstrate the superior properties imparted by the high-low aging treatment of the invention, as compared with the standard one-step aging treatment. They show that all specimens that had received the high-low aging treatment of the invention exhibited a pitting type of corrosion attack. The control specimens were more susceptible to intergranular corrosion.

TABLE 3  
[Corrosion depth in mils]

| Dia. (in.)  | Standard Aging |      |         | High-Low Aging |      |      |
|-------------|----------------|------|---------|----------------|------|------|
|             | Avg.           | Max. | Type    | Avg.           | Max. | Type |
| 2.500-----  | 3.7            | 7.3  | P and I | 3.6            | 7.5  | P    |
| 2.5625----- | 5.1            | 6.8  | P and I | 3.2            | 4.7  | P    |
| 2.8750----- | 4.2            | 7.0  | P and I | 2.9            | 4.7  | P    |
| 3.00-----   | 5.5            | 9.0  | P and I | 2.9            | 5.8  | P    |
| 3.125-----  | 4.3            | 8.2  | P and I | 2.9            | 5.8  | P    |
| 3.250-----  | 4.6            | 7.1  | P and I | 2.4            | 4.7  | P    |
| 3.500-----  | 4.5            | 7.2  | P and I | 2.3            | 4.5  | P    |

P, Pitting; I, Intergranular—Attack.

#### EXAMPLE 3

A 3½" diameter rod of alloy 2017-T4 was cut into standard tensile and corrosion test specimens. The alloy had the chemical composition: Si 0.52, Fe 0.55, Cu 3.74, Mn 0.61, Mg 0.65, balance substantially Al.

The specimens were aged at 450° F. for 2 hours, followed by aging at 325° F. for 4 hours. The mechanical properties were tested while the corrosion specimens were subjected to the standard  $\text{NaCl}-\text{H}_2\text{O}_2$  accelerated test described above. Average and maximum values and type of corrosion were determined.

The specimens tested typically showed a tensile strength (k.s.i.) of 58.7, a yield strength (k.s.i.) of 46.0, and elongation of 13%. The corrosion depth in mils was 3.7 average, 10.2 maximum. The corrosion was entirely of the pitting type.

#### EXAMPLE 4

##### *High-low aging of alloy 7075*

In order to illustrate the applicability of the high-low aging treatment to other alloy systems, samples of zinc-bearing alloy 7075 rod in solution heat treated condition were aged, and standard tensile and corrosion test specimens were tested as described previously. The high-low aging practices used and the results obtained are compared in Table 4 with the results obtained by conventional aging practice at 245–255° F. for 24 hours.

TABLE 4

| Aging Practice                             | Corrosion Depth (mils) |      |      | Properties |      |    |
|--------------------------------------------|------------------------|------|------|------------|------|----|
|                                            | Avg.                   | Max. | Type | TS         | YS   | EL |
| 250° F., 24 hrs. (Standard)-----           | 6.1                    | 9.1  | I    | 79.6       | 73.4 | 11 |
| 350° F., 5 hrs., plus 275° F., 10 hrs----- | 2.8                    | 3.4  | P    | 78.7       | 68.7 | 13 |
| 350° F., 5 hrs., plus 250° F., 10 hrs----- | 4.5                    | 6.7  | P    | 77.5       | 66.0 | 12 |
| 350° F., 5 hrs., plus 250° F., 15 hrs----- | 1.8                    | 2.4  | P    | 75.0       | 64.5 | 13 |

The comparison shows that high-low aging practices can be employed to substantially eliminate intergranular corrosion, with only a slight reduction in mechanical properties.

The aging practice of the present invention may follow conventional preparation of the alloy in solution heat treated condition, after which the alloy is heated from substantially ambient temperature to a suitable aging temperature for the initial aging step previously discussed. The temperature is maintained for a substantial proportion of the total aging time, not less than about one hour. The subsequent lower temperature aging step accounts for at least half (e.g. about 50-90%) of the total aging time.

The expressions "copper-bearing" and "zinc-bearing" aluminum base alloys are used herein to specify alloys which are predominantly aluminum and contain, respectively, copper and zinc as their major alloying addition, which is consistent with Aluminum Association designations for the 2000 and 7000-series alloys.

The published composition limits for various commercial alloys discussed herein are given below:

|                    | 2624          | 2017          | 7075           |  |
|--------------------|---------------|---------------|----------------|--|
| Si.....            | 0.50 max..... | 0.8 max.....  | 0.50 max.....  |  |
| Fe.....            | 0.50 max..... | 1.0 max.....  | 0.7 max.....   |  |
| Cu.....            | 3.8-4.9.....  | 3.5-4.5.....  | 1.2-2.0.....   |  |
| Mn.....            | 0.30-0.9..... | 0.40-1.0..... | 0.30 max.....  |  |
| Mg.....            | 1.2-1.8.....  | 0.20-0.8..... | 2.1-2.9.....   |  |
| Cr.....            | 0.10 max..... | 0.10 max..... | 0.18-0.40..... |  |
| Zn.....            | 0.25 max..... | 0.25 max..... | 5.1-6.1.....   |  |
| Ti.....            |               |               | 0.20 max.....  |  |
| Others, each.....  | .05.....      | .05.....      | .05.....       |  |
| Others, Total..... | 0.15.....     | 0.18.....     | 0.15.....      |  |
| Al.....            | Balance.....  | Balance.....  | Balance.....   |  |

While present preferred examples of the practice of the invention have been described, it will be understood that the invention may be otherwise variously embodied and practiced within the scope of the following claims.

What is claimed is:

1. The method of treating a copper-bearing aluminum base alloy so as to reduce its tendency toward the development of intergranular corrosion in the aged condition, comprising the steps of: providing the alloy in solution heat treated condition, substantially at room temperature, heating the solution treated alloy to an aging temperature of about 400° F., maintaining said temperature for about 3 hours, cooling the alloy to a lower temperature of about 300° F., and aging the alloy at said lower temperature for about 10 hours.

2. The method of treating a copper-bearing aluminum base alloy so as to reduce its tendency toward the development of intergranular corrosion in the aged condition, comprising the steps of: providing the alloy in solution heat treated condition, substantially at room temperature, heating the solution treated alloy to an aging temperature of about 450° F., maintaining said temperature for about 2 hours, cooling the alloy to a lower temperature of about 325° F., and aging the alloy at said lower temperature for about 4 hours.

3. The method of treating a zinc-bearing aluminum base alloy so as to reduce its tendency toward the development of intergranular corrosion in the aged condition, comprising the steps of: providing the alloy in solution heat treated condition, substantially at room temperature, heating the solution treated alloy to an aging

45

period constituting about 10% to about 50% of the total aging time in said first and second aging periods.

6. The method of claim 5, wherein said first aging period constitutes about one-third of the total aging time.

7. The method of treating a copper-bearing aluminum base alloy in accordance with claim 5, including the steps of maintaining the alloy during said first aging period in the temperature range of about 375-475° F., and thereafter maintaining the alloy during said second aging period in the temperature range of about 275-350° F.

8. The method of treating a copper-bearing aluminum base alloy in accordance with claim 5, said alloy containing not more than 0.5% silicon, by weight, including the steps of maintaining the alloy during said first aging period for about 3 hours in the temperature range of 375-425° F., and thereafter maintaining the alloy during said second aging period for about 10 hours in the temperature range of 275-325° F.

9. The method of treating a zinc-bearing aluminum base alloy in accordance with claim 5, including the steps of maintaining the alloy during said first aging period for about 5 hours in the temperature range of 325°-400° F., and thereafter maintaining the alloy during said second aging period for about 10 hours in the temperature range of 200-300° F.

10. The method of treating a zinc-bearing aluminum base alloy in accordance with claim 5, said alloy containing 5.1 to 6.1% zinc, 2.1 to 2.9% magnesium and 1.2 to 2.0% copper, by weight, including the steps of maintaining the alloy during said first aging period at about 350° F. for approximately 5 hours, and, during said second aging period, at about 250° F.

11. The method of treating a copper-bearing aluminum base alloy in accordance with claim 5, said alloy containing 3.8 to 4.9% copper, 1.2 to 1.8% magnesium and

temperature of about 350° F., maintaining said temperature for about 5 hours, cooling the alloy to a lower temperature of about 250° F., and aging the alloy at said lower temperature for about 10 hours.

5. In the treatment of aluminum alloys which are susceptible to solution heat treatment and artificial aging, the method of treating a copper-bearing or zinc-bearing aluminum base alloy of the type which exhibits a tendency toward the development of intergranular corrosion following constant-temperature aging, comprising the steps of: providing the alloy in solution heat treated condition, by heating said alloy in the temperature range from about 840 to about 1050° F. for sufficient time to dissolve the soluble constituents and thereafter quenching the alloy substantially to room temperature; heating the solution treated alloy to an aging temperature in the range from about 325° F. to about 475° F., and maintaining said temperature substantially constant in a first aging step for a period of time representing about one-third of the total aging time; and completing the aging

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

491

0.30 to 0.9% manganese, by weight, including the steps of maintaining the alloy during said first aging period at about 400° F. for approximately 3 hours, and, during said second aging period, at about 300° F.

12. The method of treating a copper-bearing aluminum base alloy in accordance with claim 5, said alloy containing 3.5 to 4.5% copper, 0.4 to 1.0% manganese and 0.20 to 0.8% magnesium, by weight, including the steps of maintaining the alloy during said first aging period at about 450° F. for approximately 2 hours, and, during 10 said second aging period, at about 325° F.

## References Cited by the Examiner

## UNITED STATES PATENTS

|           |        |                  |            |
|-----------|--------|------------------|------------|
| 2,159,010 | 5/1939 | Dix et al. ----- | 148—159    |
| 2,242,944 | 5/1941 | Dix et al. ----- | 148—159    |
| 3,133,839 | 5/1964 | Thomas -----     | 148—11.5 X |

## FOREIGN PATENTS

432,815 12/1936 Great Britain.

DAVID L. RECK, Primary Examiner.

C. N. LOVELL, Assistant Examiner.